

## UNITED STATES PATENT OFFICE

2,124,657

CHROMIUM PLATED ARTICLE AND METHOD  
OF PRODUCING SAME

Philip J. Ritzenthaler and Patrick J. Sheehan,  
Milwaukee, Wis., assignors to Cutler-Hammer,  
Inc., Milwaukee, Wis., a corporation of Dela-  
ware

No Drawing. Application October 11, 1934,  
Serial No. 747,888

4 Claims. (Cl. 204—13)

This invention relates to chromium plated articles and a method of producing such articles.

An object of the invention is to provide a chromium surface of a very high lustre.

5 Another object is to provide a simple and inexpensive method for producing a chromium deposit of high lustre.

Another object is to provide a chromium deposit which affords a maximum protection from 10 corrosion.

Another object is to provide a method of chromium plating which entails a minimum amount of material, labor, and time for a given thickness of protective coating.

15 Another object is to provide an efficient method of chromium plating for die castings.

Another object is to provide a dipping solution suitable for employment in the production of chromium deposits of the aforementioned character.

20 Other objects and advantages will hereinafter appear.

In the heretofore known method of chromium plating of articles, a base surface was first polished to the desired smoothness. Thereafter, a heavy layer of copper was deposited on said surface and the copper deposit was again polished to a high lustre. Thereupon a coating of nickel was deposited on the polished copper, and the 25 nickel in turn was polished to high lustre, after which a coating of chromium was deposited on the nickel. This chromium layer then presented a surface of high lustre. This process is very wasteful in material, labor, and time, on account 30 of the repeated polishing operations required for the intermediate layers of metal. Relatively thick coats of the various metals must be deposited so as to leave a sufficient amount after the polishing operation has removed some of the 35 metal. The repeated polishing consumes considerable time and labor, all of which makes the plating of chromium expensive.

The chromium plating of die-cast articles which are made of an alloy having a zinc base 40 was particularly unsatisfactory, because it is practically impossible or at least very difficult to deposit a well-adhering layer of copper on the die metal with the result that the finished chromium plated article peels and soon loses its good appearance.

45 The method of plating which is the subject of the present invention avoids the necessity of polishing the intermediate layers of metal and yet results in a bright chromium surface of high lustre. The method is also particularly suitable

for the plating of articles made of die casting metals. It produces thereon the same high lustre of the chromium coating as is produced on articles made of other metals, and affords better protection against corrosion than prior methods. 5

In accordance with the present invention, the article which is to be provided with a chromium surface is first electroplated with a layer of cadmium. The cadmium is then dipped in a suitable brightening solution, whereupon a layer of 10 nickel and thereafter a layer of chromium is deposited thereon. With this process it is only necessary to polish the base, while no polishing operations are required after the deposition of the intermediate metal layers. The resulting 15 surface has a very high lustre, which is only equalled with the old method by the exercise of the utmost care during every step.

The process is preferably carried out in the following manner:

20 The article which is to be chromium plated is thoroughly cleaned and polished to the desired smoothness. Thereafter it is plated in the usual manner with a layer of cadmium. The cadmium plating bath should have a concentration of 2 25 to 3 ounces of metallic cadmium per gallon of solution.

After the cadmium has been deposited the article is preferably dipped into a solution of 5 to 10% of acetic acid and .5% iodine, having added 30 thereto 2 to 5% of potassium iodide as a stabilizing agent. This dip produces a bright lustrous surface on the cadmium. The dipping may be prolonged for any length of time, provided that the cadmium layer previously deposited is not 35 completely removed from the base surface. Hence, the process does not require extreme care when carried out. The resulting cadmium surface is an exact duplicate of the polished surface of the base, but having even a higher lustre than the latter. Thereafter the article is washed in water and then put into the nickel bath. The layer of nickel which is deposited need only be very thin. After again washing the article it is plated with a layer of chromium by the usual 40 method.

The final chromium surface is bright and of high lustre and reflecting power.

In the above described solution, bromine may 45 be substituted for the iodine as follows:

Acetic acid 5-10%, bromine .1 to .2%, hydrochloric acid .5% and postassium bromide 2 to 5%.

The process when using the bromine solution is the same as that used when employing the 55

iodine solution. It will be understood that wherever in the appended claims iodine or iodide is specified, bromine and bromide, respectively and of the proper concentration as described, 5 may be substituted.

5 Dipping solutions for producing a relatively bright surface on cadmium plated ware have been known heretofore, but most of these solutions were not suitable for chromium plating, while 10 others produced a metal surface of insufficient lustre to insure a mirror-like surface on the subsequently deposited chromium. Hence it has always been found necessary heretofore to polish the intermediate metal deposits. A dipping solution 15 which has been used in the past to produce a high lustre on cadmium consists of chromic acid and sulphuric acid in which the ratio of chromic acid to sulphur acid radical is between 20:1 and 40:1. However, this solution 20 leaves a chromate film which has been formed during the chromic acid dip,—which film prevents a good adherence of the subsequent metal layers to the cadmium and retention of the original lustre. We have found that by following 25 the chromium dip aforescribed with another dip of short duration in a hydrochloric acid solution, the film is removed. The article is thereafter washed in water and then put into the nickel bath and the subsequent treatment is the 30 same as that aforescribed in connection with the iodine dip.

What we claim as new and desire to secure by Letters Patent is:

1. An electroplated chromium finished article 35 having a natural high lustre, which comprises a cadmium electroplated smooth base, the cadmium surface thereof being chemically brightened but

being otherwise in original condition, a natural high lustre nickel coating electrodeposited directly on such cadmium surface and a chromium coating electrodeposited on such nickel coating.

2. An electroplated chromium finished article 5 consisting of a smooth base and electrodeposited coatings therefor of chromium on nickel on cadmium, each coating being left in original condition save for chemical brightening of the cadmium coating, and the nickel and chromium 10 coatings each having a natural surface of high lustre.

3. In a process of electroplating a base having a smooth surface, the steps of electrodepositing on the base a layer of cadmium, dipping the 15 cadmium coated base in an acetic acid solution containing one of the group consisting of iodine and bromine to obtain a high lustre surface, electrodepositing on the cadmium a layer of nickel and electrodepositing on the nickel a layer 20 of chromium to obtain a chromium surface of high lustre, all without any mechanical polishing or any dipping other than that specified.

4. In a process of electroplating a base having a smooth surface, the steps of depositing on the 25 base a layer of cadmium, finishing the cadmium for high surface lustre while preserving a layer of the cadmium by dipping into an acetic acid solution containing a halogen, electrodepositing on the dipped cadmium a layer of nickel having 30 a natural surface of high lustre and electrodepositing on the natural surface of the nickel a layer of chromium having a natural surface of high lustre.

PHILIP J. RITZENTHALER.  
PATRICK J. SHEEHAN.